

April 20, 1926.

1,581,443

J. C. HENDERSON

HEAT RESISTING ARTICLE

Filed April 9, 1925

2 Sheets-Sheet 1



J. C. Henderson  
INVENTOR  
BY  
Bartlett Howard  
ATTORNEY

April 20, 1926.

1,581,443

J. C. HENDERSON

HEAT RESISTING ARTICLE

Filed April 9, 1925

2 Sheets-Sheet 2



F-14 8



F-14 10



F-14 9

J. C. Henderson INVENTOR  
Bartholomew & Brown ATTORNEYS

## UNITED STATES PATENT OFFICE.

JOHN CLIFTON HENDERSON, OF NEW YORK, N. Y., ASSIGNOR TO DRIVER-HARRIS COMPANY, OF HARRISON, NEW JERSEY, A CORPORATION OF NEW JERSEY.

## HEAT-RESISTING ARTICLE.

Application filed April 9, 1925. Serial No. 21,749.

To all whom it may concern:

Be it known that I, JOHN C. HENDERSON, a citizen of the United States, residing at New York, county of New York, State of New York, have invented a certain new and useful Improvement in Heat-Resisting Articles, of which the following is a full, clear, and exact description.

My invention relates to heat resisting articles which when in use are subjected from time to time to high external temperatures and has for its object to provide means for reenforcing such articles so as to enable them to withstand to a higher degree the strains due to the repeated heating and cooling to which they are subjected.

Articles such as boxes, box covers, retorts and other castings have for some time past been made of heat resisting alloys and used with remarkable success. It has been found, however, that on account of the repeated heating and cooling to which they are subjected these articles, more particularly when they have thickened rims or other projections, or angles, sometimes fail by cracking, thereby reducing their life to a very considerable degree. Where there is a rim or projection joining the body of the article the cracking is most liable to occur at the joint. Furthermore, it is known that in casting such articles there is sometimes formed during the casting process what are known as "draws", the same being slight cracks due to the shrinking of the metal, which cracks during the repeated heatings and coolings are apt to grow so as to cause the article to give way. In order to avoid these difficulties I have reenforced such articles at points where these defects are likely to develop by a wrought rod of approximately similar material embedded in and connected to the cast material by local welds.

Thus if the body of the article is made of a heat resisting nickel-chromium-iron alloy, the reenforcing rod is also made of a heat resisting nickel-iron-chromium alloy. If made of chrome-iron or silicon-iron the reenforcing rods are made of chrome or silicon iron respectively. I preferably make the body of the articles of a nickel-chromium iron alloy having about 60% nickel, 12% chromium and 27% iron, and make the wrought reenforcing member of the mate-

rial having substantially the same composition.

The following is a description of an embodiment of my invention, reference being had to the accompanying drawings, in which:

Fig. 1 is a plan view of a box embodying my invention;

Fig. 2 is a section of the same on the line 2—2, Fig. 3;

Fig. 3 is a vertical section;

Figs. 4 and 5 are enlarged sectional details;

Fig. 6 shows a horizontal section of a modification on the line 6—6, Fig. 7;

Fig. 7 shows a vertical section on the line 7—7, Fig. 6;

Fig. 8 shows an enlarged sectional detail on the line 8—8, Fig. 7;

Fig. 9 is a modified embodiment of my invention comprising a circular box and cover;

Fig. 10 is a section on the line 10—10, Fig. 9; and

Fig. 11 is a section of the cover on the line 11—11, Fig. 9.

Referring more particularly to the drawings, 2 is the cast body portion of a rectangular carburizing box or mouthed container made of a heat resisting alloy and having at its upper end a projecting rim or bead 4 and at its lower end supporting feet 6. Embedded in the cast body of the box at its upper rim is a rod 8 of wrought material of similar composition to that composing the body of the box, while embedded in bottom portions of the box and extending into the feet are short wrought rod sections 10 of similar material.

The reenforcing member 8 in the rim extends around the mouth of the box but is preferably interrupted at two diametrical points so as to form two sections, each section having portions lying upon three sides of the box, as shown. The reenforcing member 8 is made in two sections, since in connection with a rectangular box it is difficult to make a rod made of one section lie in a given plane so as to be properly located within the rim.

When the box is relatively tall I also embed in the central portion of the side wall a flat strip of approximately similar

wrought material connected to the cast mass by a weld. This may be a strip of wire mesh as shown at 12.

Figs. 6, 7 and 8 show a rectangular box 5 made of heat resisting alloy having at each of its corners a wrought angular plate 14 plate 14 of similar alloy, preferably perforated, which is embedded in the cast mass 16 and welded to the same reenforcing the 10 corner portions.

In Figs. 9, 10 and 11 a round box is shown having a wrought hoop-like reenforcing member 18 of heat resisting alloy similar to the cast body portion 20 of the box, and 15 wrought reenforcing members 22 in the feet. In this case the circular reenforcing member 18 is preferably made in the form of a closed loop, as shown.

The wrought members are in each instance 20 welded to the cast mass. The rim rods for boxes having half inch walls and three-quarters of an inch thick at the rims I preferably make about three eights of an inch thick and the other reenforcing members 25 of similar relative thickness.

Figs. 9 and 11 show a box cover 24 having a handle 26, the cover and outer portion of the handle being cast integral and of heat resisting alloy, and the handle having embedded 30 therein a wrought rod 28 of substantially similar alloy which also extends into the body of the cover and has its surface welded to the adjacent cast portions of cover and handle.

In producing the articles above referred to, the reenforcing members are placed in the molds, being supported in proper positions by chaplets of similar material, and the alloy for the body of the article is then 40 heated to a point sufficiently high to fuse the surface of the wrought members slightly when poured about them so as to form a weld between the surface of the wrought member of the cast body portion, thus establishing an intimate connection between the 45 two.

The flat strip of Fig. 3 is provided with holes and when sheet metal portions, as in 50 Figs. 6, 7 and 8 are employed, I preferably perforate them so as to form clinch holes, thus forming a still more intimate connection between the reenforcing members and the cast body of the mass.

The wrought members of the character referred to are usually produced by rolling or drawing and when so produced have a higher tensile strength than castings of the same alloy and a greater elasticity. In all cases the wrought portions are cleaned so that they 55 are in condition to make a good weld.

Where the nickel-chromium-iron alloy, particularly above referred to, is used, the pouring temperature of that alloy is approximately 65 2900 degrees Fahrenheit, and in

carrying out my invention I heat the portion of the alloy to be cast to substantially 2900 degrees Fahrenheit or slightly higher than the pouring temperature, which is several hundred degrees Fahrenheit above the melting point of the wrought reenforcing members and results in forming a weld between the cast portion and the surface of the wrought rod. The presence of the wrought members in the mold results in producing 70 what is known as a "chill" in the cast metal surrounding them. These "chilled" portions are of finer texture and greater tensile strength than the unchilled cast portions so that the reenforcing members strengthen the 75 article not only on account of their own characteristics but also on account of their action on the metal being cast. The articles have reenforcing internal "chills" at the points of strain coacting with the reenforcing 80 members.

As will be evident to those skilled in the art, my invention permits of various modifications without departing from the spirit 85 thereof or the scope of the appended claims. 90

What I claim is:

1. A container subjected when in use to high external temperatures, having a body portion comprising a cast mass of high heat resisting alloy and a wrought reenforcing 95 and strain resisting member of similar alloy embedded in said mass, there being a weld between said cast mass and said wrought member, the exterior wall of said container having an angle and said wrought member being angular and extending around said angle within said wall. 100

2. An article subjected when in use to high external temperatures constituting a mouthed container having a body portion comprising a cast mass of high heat resisting alloy and a wrought reenforcing and strain resisting member of similar alloy embedded in said mass adjacent to the mouth of said container and extending continuously along 105 more than one side thereof, there being a weld between said cast mass and said wrought member. 110

3. An article subjected when in use to high external temperatures, constituting a mouthed container having a body portion comprising a cast mass of high heat resisting alloy and a wrought reenforcing and strain resisting member of similar alloy embedded 115 in said mass adjacent to the mouth of said container, there being a weld between said cast mass and said wrought member, the mouth of said container being rectangular and said member being divided into two 120 parts, each part having portions on three sides of said mouth. 125

4. A container subjected when in use to high external temperatures having an outwardly projecting flange adjacent to its mouth and entirely surrounding the same 130

forming a thickened portion, said container comprising a cast mass of high heat resisting alloy and having a wrought reinforcing and strain resisting member of similar alloy embedded in said thickened portion, there being a weld between said cast mass and said wrought member, the mouth of said con-

tainer having an angle and said wrought member being angular and extending around said angle.

In testimony whereof, I have signed my name to this specification this 26th day of March, 1925.

JOHN CLIFTON HENDERSON.